# EUROPEAN PATENT SPECIFICATION

(11) **EP 3 628 724 B1**
(45) Date of publication and mention of the grant of the patent: **28.07.2021**
(21) Application number: 18196604.5
(22) Date of filing: 25.09.2018
(51) Int. Cl.: C11D 3/37, C11D 11/02

(54) **POWDER AND GRANULE, PROCESS FOR MAKING SUCH POWDER AND GRANULE, AND USE THEREOF**
PULVER UND GRANULAT, VERFAHREN ZUR HERSTELLUNG SOLCH EINES PULVERS UND GRANULATS UND VERWENDUNG DAVON
POUDRES ET GRANULÉS, PROCÉDÉ DE FABRICATION DE CES POUDRES ET GRANULÉS ET LEUR UTILISATION

(43) Date of publication of application: 01.04.2020
(73) Proprietor: BASF SE, 67056 Ludwigshafen am Rhein (DE); Henkel AG & Co. KGaA, 40589 Düsseldorf (DE)
(72) Inventor: Ettl, Roland, 67056 Ludwigshafen (DE); Pirrung, Frank, 67056 Ludwigshafen (DE); Gebert-Schwarzwaelder, Antje, 41469 Neuss (DE); Bluhm, Nadine, 40233 Düsseldorf (DE); Junkes, Christa, 40595 Düsseldorf (DE); Herbst, Daniela, 40589 Düsseldorf (DE); Giesen, Brigitte, 40589 Düsseldorf (DE)
(74) Representative: BASF IP Association

(56) References cited:
- EP-A1- 3 196 284
- WO-A1-2015/078736
- WO-A1-2016/049456
- WO-A1-2018/028935

## Description

The present invention is directed towards a process for making a powder or granule containing
(A) at least one copolymer obtainable by polymerization of at least one monomer according to formula (I): in an amount of 1 to 70 mole%,
   wherein n is ≥ 3
   and
   at least one monomer according to formula (II): in an amount of 30 to 99 mole%,
(B) at least one homo- or copolymer of (meth)acrylic acid, partially or fully neutralized with alkali,
   wherein the weight ratio of (A) to (B) is from 20:80 to 80:20,
   said process comprising the steps of
   (a) mixing the at least one copolymer (A) and the at least one homo- or copolymer in the presence of water,
   (b) removing most of said water by spray-drying or spray granulation using a gas with an inlet temperature of at least 125°C.

Granules have the advantage of being highly concentrated, with a low amount of residual water. That means that in case of shipping, almost no water has to be shipped, and costs for extra weight can be avoided.

The soil release agents based on (meth)acrylic esters for use preferably in liquid detergents are known from WO 2015/078736.

Soil release agents known from WO 2015/078736 do not crystallize upon drying and therefore they cannot be transferred into granules or powders.

Other processes for making a powder or a granule not according to the current invention are disclosed in patent document EP3196284 A1.

It was an objective of the present invention to provide a copolymer in form of a powder or of a granule for powder detergents, stable under high alkaline conditions with no malodour formation and evolvement during storage conditions. It was further an objective to provide a process for making a copolymer in form of a powder or of a granule, such powder or granule stable under high alkaline conditions with no malodour formation and evolvement during storage conditions. Accordingly, the process defined at the outset has been found, hereinafter also being referred to as "inventive process" or as "process according to the (present) invention".

The inventive process provides granules or powders, hereinafter also referred to as "inventive granules" or "inventive powders", respectively. Inventive powders and inventive granules can be manufactured according to the inventive process.

In the course of the present invention, inventive powders are particulate materials that are solids at ambient temperature and that preferably have an average particle diameter in the range of from 0.001mm to less than 2.5 mm, preferably 0,1mm up to 1 mm. The average particle diameter of inventive powders can be determined, e.g., by LASER diffraction methods, for example with Malvern apparatus, and refers to the volume average. Inventive granules are particulate materials that are solids at ambient temperature and that preferably have an average particle diameter in the range of from 0.1 mm to 2 mm, more preferably between 0.45 mm to 1.00 mm. The average particle diameter of inventive granules can be determined, e.g., by optical or preferably by sieving methods. Sieves employed may have a mesh in the range of from 60 to 1,250 µm.

In one embodiment of the present invention, inventive powders or inventive granules have a broad particle diameter distribution. In another embodiment of the present invention, inventive powders or inventive granules have a narrow particle diameter distribution. The particle diameter distribution can be adjusted, if desired, by multiple sieving steps.

Granules and powders may contain residual moisture, moisture referring to water including water of crystallization and adsorbed water. The amount of water may be in the range of from 0.1 to 20% by weight, preferably 1 to 15% by weight, referring to the total solids content of the respective powder or granule, and may be determined by Karl-Fischer-titration or by drying at 160°C to constant weight with infrared light.

Particles of inventive powders may have regular or irregular shape. Preferred shapes of particles of inventive powders are spheroidal shapes.

Powders and granules made according to the inventive process contain
(A) at least one copolymer obtainable by polymerization of at least one monomer according to formula (I): in an amount of 1 to 70 mole%,
   wherein n is ≥ 3
   and
   at least one monomer according to formula (II): in an amount of 30 to 99 mole%, also being referred to as "copolymer (A)",
(B) at least one homo- or copolymer of (meth)acrylic acid, partially or fully neutralized with alkali, hereinafter also referred to as "polymer (B)". Polymers (B) that are homopolymers are also being referred to as "homopolymers (B)", and polymers (B) that are copolymers are also being referred to as "copolymers (B)",
wherein the weight ratio of (A) to (B) is from 20:80 to 80:20.

Another aspect of the present invention, powders and granules made according to the inventive process contain
(A) in the range of from 40 - 75 % by weight of at least one copolymer obtainable by polymerization of at least one monomer according to formula (I): in an amount of 1 to 70 mole%,
   wherein n is ≥ 3
   and
   at least one monomer according to formula (II): in an amount of 30 to 99 mole%,
(B) in the range of from 60 - 25 % by weight of at least one homo- or copolymer of (meth)acrylic acid, partially or fully neutralized with alkali,
percentages referring to the solids content of said powder or granule.

In the context of the present invention, a copolymer (A) is obtainable by polymerization of at least one monomer according to formula (I): in an amount of 1 to 70 mole%,
wherein n is ≥ 3
and
at least one monomer according to formula (II): in an amount of 30 to 99 mole%.

In a preferred embodiment, n of the monomer according to formula (I) is between 3 and 120, preferably between 5 and 50, more preferably between 5 and 46 and even more preferably between 5 and 23.

In another preferred embodiment, n of the monomer according to formula (I) is selected from the group consisting of 7, 23 and 46.

In a further preferred embodiment, the monomer according to formula (I) is present in the amount of 5 to 70 mole% and the monomer according to formula (II) is present in the amount of 30 to 95 mole%. In a more preferred embodiment, the monomer according to formula (I) is present in the amount of 9 to 70 mole% and the monomer according to formula (II) is present in the amount of 30 to 91 mole%. In an even more preferred embodiment, the monomer according to formula (I) is present in the amount of 9 to 67 mole% and the monomer according to formula (II) is present in the amount of 33 to 91 mole%. In another preferred embodiment, the monomer according to formula (I) is present in the amount of 5 to 60 mole% and the monomer according to formula (II) is present in the amount of 40 to 95 mole%. In a further preferred embodiment, the monomer according to formula (I) is present in the amount of 5 to 50 mole% and the monomer according to formula (II) is present in the amount of 50 to 95 mole%. In a further preferred embodiment, the monomer according to formula (I) is present in the amount of 1 to 67 mole% and the monomer according to formula (II) is present in the amount of 33 to 99 mole%

The copolymer (A) can be produced by polymerization. More precisely it can be prepared by using known polymerization methods as described, for example, in WO 2015/078736 or in US 4,170,582, US 2009/0234062 or US 7,687,554, as exemplified for emulsion and miniemulsion polymerizations, but without use of surfactants.

Polymer (B) is selected from homopolymers (B) of (meth)acrylic acid and of copolymers (B) of (meth)acrylic acid, preferably of acrylic acid, partially or fully neutralized with alkali. In the context of the present invention, copolymers (B) are those in which at least 50 mol-% of the comonomers are (meth)acrylic acid, preferably at least 75 mol-%, even more preferably 80 to 99 mol-%.

Suitable comonomers for copolymers (B) are ethylenically unsaturated compounds, such as styrene, isobutene, ethylene, α-olefins such as propylene, 1-butylene, 1-hexene, and ethylenically unsaturated dicarboxylic acids and their alkali metal salty and anhydrides such as but not limited to maleic acid, fumaric acid, itaconic acid disodium maleate, disodium fumarate, itaconic anhydride, and especially maleic anhydride. Further examples of suitable comonomers are C₁-C₄-alkyl esters of (meth)acrylic acid, for example methyl acrylate, methyl methacrylate, ethyl acrylate, ethyl methacrylate, n-butyl acrylate.

In one embodiment of the present invention, polymer (B) is selected from copolymers of (meth)acrylic acid and a comonomer bearing at least one sulfonic acid group per molecule. Comonomers bearing at least one sulfonic acid group per molecule may be incorporated into polymer (B) as free acid or least partially neutralized with alkali. Particularly preferred sulfonic-acid-group-containing comonomers are 1-acrylamido-1-propanesulfonic acid, 2-acrylamido-2-propanesulfonic acid, 2-acrylamido-2-methylpropanesulfonic acid (AMPS), 2-methacrylamido-2-methylpropanesulfonic acid, 3-methacrylamido-2-hydroxypropanesulfonic acid, allylsulfonic acid, methallylsulfonic acid, allyloxybenzenesulfonic acid, methallyloxybenzenesulfonic acid, 2-hydroxy-3-(2-propenyloxy)propanesulfonic acid, 2-methyl-2-propene-1-sulfonic acid, styrenesulfonic acid, vinylsulfonic acid, 3-sulfopropyl acrylate, 2-sulfoethyl methacrylate, 3-sulfopropyl methacrylate, sulfomethacrylamide, sulfomethylmethacrylamide, and salts of said acids, such as the sodium salts, potassium salts or ammonium salts thereof.

Copolymers (B) may be selected from random copolymers, alternating copolymers, block copolymers and graft copolymers, alternating copolymers and especially random copolymers being preferred.

Useful copolymers (B) are, for example, copolymers of acrylic acid and methacrylic acid, copolymers of acrylic acid and maleic anhydride, ternary copolymers of acrylic acid, methacrylic acid and maleic anhydride, random or block copolymers of acrylic acid and styrene, copolymers of acrylic acid and methyl acrylate. More preferred are homopolymers of methacrylic acid. Even more preferred are homopolymers of acrylic acid.

Polymer (B) may constitute straight-chain or branched molecules. Branching in this context will be when at least one repeating unit of such polymer (B) is not part of the main chain but forms a branch or part of a branch. Preferably, polymer (B) is not cross-linked.

In one embodiment of the present invention, polymer (B) has an average molecular weight M_{w} in the range of from 1,200 to 30,000 g/mol, preferably from 2,500 to 15,000 g/mol and even more preferably from 3,000 to 10,000 g/mol, determined by gel permeation chromatography (GPC) and referring to the respective free acid.

In one embodiment of the present invention, polymer (B) is at least partially neutralized with alkali, for example with lithium or potassium or sodium or combinations of at least two of the forgoing, especially with sodium. For example, in the range of from 10 to 100 mol-% of the carboxyl groups of polymer (B) may be neutralized with alkali, especially with sodium.

In one embodiment of the present invention, polymer (B) is selected from per-sodium salts of polyacrylic acid, thus, polyacrylic acid, fully neutralized with sodium.
In one embodiment of the present invention, polymer (B) is selected from a combination of at least one polyacrylic acid and at least one copolymer of (meth)acrylic acid and a comonomer bearing at least one sulfonic acid group per molecule, both polymers being fully neutralized with alkali.

In one embodiment of the present invention, polymer (B) is selected from per-sodium salts of polyacrylic acid with an average molecular weight M_{w} in the range of from 1,200 to 30,000 g/mol, preferably from 2,500 to 15,000 g/mol and even more preferably from 3,000 to 10,000 g/mol, determined by gel permeation chromatography (GPC) and referring to the respective free acid.

The inventive process comprises two steps,
(a) mixing the at least one copolymer (A) and the at least one homo- or copolymer (B) in the presence of water,
(b) removing most of said water by spray-drying or spray granulation,
hereinafter also referred to as step (a) and step (b). Usually, step (b) is performed after step (a).

Step (a) and step (b) will be described in more detail below.
Mixing of copolymer (A) and polymer (B) is usually performed in the presence of water. Said mixing can be conducted in a way that an aqueous solution of polymer (B) and an aqueous solution of copolymer (A) are being combined in a vessel, preferably under stirring. It is also possible to combine an aqueous solution of polymer (B) and solid copolymer (A), or to combine an aqueous solution of copolymer (A) with solid polymer (B), or to combine aqueous slurries of copolymer (A) and polymer (B). In an alternative embodiment, water is provided and subsequently, polymer (B) and then copolymer (A) are added. In a preferred embodiment, a solution of copolymer (A) is provided that has a temperature of 35 to 75°C, and polymer (B) is being added, either in bulk or as solution, under stirring.

Step (a) can be performed at ambient temperature. In other embodiments, step (a) is being performed at 20° C or at elevated temperature, for example at a temperature in the range of from 25 to 90°C, preferably 40 to 75°C.

The water used in step (a) may be present in an amount that both copolymer (A) and polymer (B) are dissolved. However, it is also possible to use less amounts of water and mix copolymer (A) and polymer (B) in a way that a slurry is being formed. Solutions are preferred.

In one embodiment of the present invention, the total solids content of such solution or slurry formed as result of step (a) is in the range of from 20 to 75%, preferably 35 to 50%.

In one embodiment of the present invention, such solution or slurry has a pH value in the range of from 2.5 to 13, preferably from 4 to 11, and also preferably at least 5.

Mixing may be performed with mechanical support, for example shaking or stirring.

In step (b), a spray-drying or spray granulation is performed, using a gas with an inlet temperature of at least 125°C. Said gas, hereinafter also being referred to as "hot gas", may be nitrogen, a rare gas or preferably air. In the course of step (b), most of the water used in step (a) will be removed, for example at least 55%, preferably at least 65% of the water. In one embodiment of the present invention, 99% of the water at most will be removed.

Spray-drying and spray granulation will be described in more detail below.

In one embodiment of the present invention, a drying vessel, for example a spray chamber or a spray tower, is being used in which a spray-granulating process is being performed by using a fluidized bed. Such a drying vessel is charged with a fluidized bed of a solid mixture of copolymer (A) and polymer (B), obtained by any drying method such as spray drying or evaporation crystallization, and a solution or slurry of solid mixture of copolymer (A) and polymer (B) is sprayed onto or into such fluidized bed together with a hot gas stream. The hot gas inlet stream may have a temperature in the range of from 125 to 350°C, preferably 160 to 220°C.

In one embodiment of the present invention, the fluidized bed may have a temperature in the range of from 80 to 150°C, preferably 100 to 120°C.

Spraying is being performed through one or more nozzles per drying vessel. Suitable nozzles are, for example, high-pressure rotary drum atomizers, rotary atomizers, single-fluid nozzles and two-fluid nozzles, two-fluid nozzles and rotary atomizers being preferred. The first fluid is the solution or slurry obtained according to step (a), the second fluid is compressed gas, for example with a pressure of 1.1 to 7 bar.

In one embodiment of the present invention, the droplets formed during the spray-granulating have an average diameter in the range of from 10 to 500 µm, preferably from 20 to 180 µm, even more preferably from 30 to 100 µm.

In one embodiment of the present invention, the off-gas departing the drying vessel may have a temperature in the range of from 40 to 140°C, preferably 80 to 110°C but in any way colder than the hot gas stream. Preferably, the temperature of the off-gas departing the drying vessel and the temperature of the solid product present in the drying vessel are identical.

In another embodiment of the present invention, spray-granulation is being performed by performing two or more consecutive spray-drying processes, for example in a cascade of at least two spray dryers, for example in a cascade of at least two consecutive spray towers or a combination of a spray tower and a spray chamber, said spray chamber containing a fluidized bed. In the first dryer, a spray-drying process is being performed in the way as follows.

Spray-drying may be preferred in a spray dryer, for example a spray chamber or a spray tower. A solution or slurry obtained according to step (a) with a temperature preferably higher than ambient temperature, for example in the range of from 50 to 95°C, is introduced into the spray dryer through one or more spray nozzles into a hot gas inlet stream, for example nitrogen or air, the solution or slurry being converted into droplets and the water being vaporized. The hot gas inlet stream may have a temperature in the range of from 125 to 350°C.

The second spray dryer is charged with a fluidized bed with solid from the first spray dryer and solution or slurry obtained according to the above step is sprayed onto or into the fluidized bed, together with a hot gas inlet stream. The hot gas inlet stream may have a temperature in the range of from 125 to 350°C, preferably 160 to 220°C.

In one embodiment of the present invention, especially in a process for making an inventive granule, the average residence time of copolymer (A) and polymer (B), respectively, in step (b) is in the range of from 2 minutes to 4 hours, preferably from 30 minutes to 2 hours.

In another embodiment, especially in a process for making an inventive powder, the average residence time of copolymer (A) and polymer (B), in step (b) is in the range of from 1 second to 1 minute, especially 2 to 20 seconds.

In one embodiment of the present invention, the pressure in the drying vessel in step (b) is normal pressure ± 100 mbar, preferably normal pressure ± 20 mbar, for example one mbar less than normal pressure.

In one embodiment of the present invention, one or more additives (C) can be added to the solution obtained according to step (a) before performing step (b), or one or more of such additives (C) can be added at any stage during step (a). Examples of useful additives (C) are, for example, titanium dioxide, sugar, silica gel and polyvinyl alcohol. Polyvinyl alcohol in the context of the present invention refers to completely or partially hydrolyzed polyvinyl acetate. In partially hydrolyzed polyvinyl acetate, at least 95 mol-%, preferably at least 96 mol-% of the acetate groups have been hydrolyzed.

In one embodiment of the present invention polyvinyl alcohol has an average molecular weight M_{w} in the range of from 22,500 to 115,000 g/mol, for example up to 40,000 g/mol.

In one embodiment of the present invention polyvinyl alcohol has an average molecular weight Mₙ in the range of from 2,000 to 40,000 g/mol.

Additive(s) (C) can amount to 0.1 to 5 % by weight, referring to the sum of copolymer (A) and polymer (B).

Preferably, no additive (C) is being employed in step (b).
One or more additional steps (c) may be performed at any stage of the inventive proves, preferably after step (b). It is thus possible to perform a sieving step (c) to remove lumps from the powder or granule. Also, a post-drying step (c) is possible. Air classifying can be performed during or after step (b) to remove fines.

Fines, especially those with a diameter of less than 50 µm, may deteriorate the flowing behavior of powders or granules obtained according to the inventive process. However, amorphous or preferably crystalline fines may be returned to the spray vessel(s) as seed for crystallization. Lumps may be removed and either re-dissolved in water or milled and used as seed for crystallization in the spray vessel(s).

The inventive process furnishes powders or granules containing copolymer (A) and polymer (B) and, optionally, one or more additives (C). Such powders and granules exhibit overall advantageous properties including but not limited to an excellent yellowing behavior.

Another aspect of the present invention are powders and granules, hereinafter also being referred to as inventive powders or inventive granules, respectively, containing
(A) at least one copolymer obtainable by polymerization of at least one monomer according to formula (I): in an amount of 1 to 70 mole%,
   wherein n is ≥ 3
   and
   at least one monomer according to formula (II): in an amount of 30 to 99 mole%,
(B) at least one homo- or copolymer of (meth)acrylic acid, partially or fully neutralized with alkali,
   wherein the weight ratio of (A) to (B) is from 20:80 to 80:20
   in molecularly disperse form.

A further aspect of the present invention are powders and granules, hereinafter also being referred to as inventive powders or inventive granules, respectively, containing
(A) in the range of from 40 - 75 % by weight of at least one copolymer obtainable by polymerization of at least one monomer according to formula (I): in an amount of 1 to 70 mole%,
   wherein n is ≥ 3
   and
   at least one monomer according to formula (II): in an amount of 30 to 99 mole%,
(B) in the range of from 60 - 25 % by weight of at least one homo- or copolymer of (meth)acrylic acid, partially or fully neutralized with alkali,
in molecularly disperse form, percentages referring to the solids content of said powder or granule.

Copolymer (A) and polymer (B) have been defined above.

In the context of the present invention, the term "in molecularly disperse form" implies that all or a vast majority, for example at least 80% of the particles of inventive powder and of inventive granules contain copolymer (A) and polymer (B).

In one embodiment of the present invention, inventive powders are selected from powders having an average particle diameter in the range of from 1 µm to less than 0.1 mm.

In one embodiment of the present invention, inventive granules are selected from granules with an average particle diameter in the range of from 0.1 mm to 2 mm, preferably 0.45 mm to 1.00 mm.

In one embodiment of the present invention, inventive powder or inventive granule contains in the range of from 20 - 80 % by weight copolymer (A) and 80 - 20 % by weight homo- or copolymer (B), percentages referring to the solids content of said powder or granule.

In a preferred embodiment of the present invention, the term "in molecularly disperse form" also implies that essentially all particles of inventive powder or inventive granule contains in the range of from 40 - 75 % by weight copolymer (A) and 60 - 25 % by weight homo- or copolymer (B), percentages referring to the solids content of the respective powder or granule.

In one embodiment of the present invention, inventive powders and inventive granules are selected from those wherein polymer (B) has an average molecular weight M_{w} in the range of from 1,200 to 30,000 g/mol, determined by gel permeation chromatography and referring to the respective free acid.

In one embodiment of the present invention, inventive powders and inventive granules are selected from those wherein copolymer (A) is a copolymer obtainable by polymerization of at least one monomer according to formula (I): in an amount of 1 to 70 mole%,
wherein n is between 5 and 7
and
at least one monomer according to formula (II): in an amount of 30 to 99 mole%.

In one embodiment of the present invention, inventive powders and inventive granules are selected from those wherein said homo- and copolymer (B) are selected from the per-sodium salts of polyacrylic acid.

In one embodiment of the present invention, inventive powders and inventive granules are selected from those wherein said polymer (B) is selected from copolymers of (meth)acrylic acid and a comonomer bearing at least one sulfonic acid group per molecule. Comonomers bearing at least one sulfonic acid group per molecule may be incorporated into polymer (B) as free acid or least partially neutralized with alkali. Particularly preferred sulfonic-acid-group-containing comonomers are 1-acrylamido-1-propanesulfonic acid, 2-acrylamido-2-propanesulfonic acid, 2-acrylamido-2-methylpropanesulfonic acid (AMPS), 2-methacrylamido-2-methylpropanesulfonic acid, 3-methacrylamido-2-hydroxypropanesulfonic acid, allylsulfonic acid, methallylsulfonic acid, allyloxybenzenesulfonic acid, methallyloxybenzenesulfonic acid, 2-hydroxy-3-(2-propenyloxy)-propanesulfonic acid, 2-methyl-2-propene-1-sulfonic acid, styrenesulfonic acid, vinylsulfonic acid, 3-sulfopropyl acrylate, 2-sulfoethyl methacrylate, 3-sulfopropyl methacrylate, sulfomethacrylamide, sulfomethylmethacrylamide, and salts of said acids, such as the sodium salts, potassium salts or ammonium salts thereof.

In one embodiment of the present invention, inventive powders and inventive granules are selected from those wherein said polymer (B) is selected from a combination of at least one polyacrylic acid and at least one copolymer of (meth)acrylic acid and a comonomer bearing at least one sulfonic acid group per molecule, both polymers being fully neutralized with alkali.

Inventive powders and inventive granules exhibit overall advantageous properties including but not limited to being stable under high alkaline conditions with no malodour formation and evolvement during storage conditions. They are therefore excellently suitable for the manufacture of cleaning agents.

Typical compact and powder detergents may for example comprise the following ingredients

The present invention is further illustrated by working examples.

General remarks: NI: Norm liter, liters under normal conditions; Nm³: norm cubic meter, cubic meter under normal conditions

### Example I: Manufacture of inventive granules

### I.1 Manufacture of spray solution SL.1

A vessel was charged with 25kg of an aqueous solution of Sokalan® PA 30 CL PN (homopolymer (B)) and 13,3kg of an aqueous solution of Sokalan® SR400 (copolymer (A)). The solution SL.1 so obtained was stirred, heated to 70°C and then subjected to spray granulation. The solid ratio between Sokalan® PA 30 CL PN and Sokalan® SR400 is 3:1.

### 1.2 Spray granulation of Spray Solution SL.1

The granulation was carried out in a lab granulator (Glatt LabSystem with Vario 3 insert attached with a zig-zag air classifier).

At the beginning, the granulator was charged with 1,3kg of solid Sokalan® PA 30 CL PN spherical particles. An amount of 200 Nm3/h of air with a temperature of 166 to 173°C was blown from the bottom. A fluidized bed of Sokalan® Pa 30 CL PN particles was obtained. The inventive solution SL.1 was introduced by spraying 7,3 kg of SL.1 (temperature of the solution: 70°C) per hour into the fluidized bed from the bottom through a two-fluid nozzle (parameters: absolute pressure in the nozzle: 5 bar). Granules were formed, and the bed temperature, which corresponds to the surface temperature of the solids in the fluidized bed, was 100°C.

Continuously, particles, which are large (heavy) enough fall through the zigzag air classifier (operated at 0,5 to 0,7 bar relative pressure) into a sample bottle. The smaller (lighter) granules were blown through the recycle back into the fluidized bed by the air classifier.

When about 1-2L of granules were collected in the sample bottle, the bottle is replaced by a new sample bottle. The collected granules were subjected to a sieving step. The mesh size of the sieve is 1mm. Two fractions were obtained: coarse particles (diameter > 1mm) and value fraction (<1mm). Coarse particles (diameter > 1mm), were milled using a hammer mill (Kinetatica Polymix PX-MFL 90D) at 4000 rpm (rounds per minute), 2 mm mesh. The powder so obtained was returned into the fluidized bed.

After 10kg of sprayed liquid a steady state was reached. The fraction <1mm was collected as inventive granule Gran 1.

In the above example, hot air can be replaced by hot nitrogen having the same temperature of 166-173°C.

### II. Manufacture of further spray solutions and spray granulation thereof

### 11.1 Manufacture of spray solution SL.2 and spray granulation

A vessel was charged with 16,67kg of an aqueous solution of Sokalan® CP 45 (Copolymer (B)) and 26,67kg of an aqueous solution of Sokalan® SR400 (copolymer (A)). The solution SL.2 so obtained was stirred, heated to 70°C and then subjected to spray granulation. The solid ratio between Sokalan® CP 45 and Sokalan® SR400 is 1:1.

For spray granulation, the protocol according to 1.2 was followed but with spraying of SL.2 instead of SL.1. Inventive granule Gran 2 was obtained.

### 11.2 Manufacture of spray solution SL.3 and spray granulation

A vessel was charged with 8,34kg of an aqueous solution of Sokalan® PA 30 CL PN (homopolymer (B)) and 13,34kg of an aqueous solution of Sokalan® SR400 (copolymer (A)). The solution SL.3 so obtained was stirred, heated to 70°C and then subjected to spray granulation. The solid ratio between Sokalan® PA 30 CL PN and Sokalan® SR400 is 1:1

For spray granulation, the protocol according to 1.2 was followed but with spraying of SL.3 instead of SL.1. Inventive granule Gran 3 was obtained.

### II.3 Manufacture of spray solution SL.4 and spray granulation

A vessel was charged with 5,22kg of an aqueous solution of Sokalan® PA 30 CL PN (homopolymer (B)) and 16kg of an aqueous solution of Sokalan® SR400 (copolymer (A)). The solution SL.4 so obtained was stirred, heated to 70°C and then subjected to spray granulation. The solid ratio between Sokalan® PA 30 CL PN and Sokalan® SR400 is 1:2

For spray granulation, the protocol according to 1.2 was followed but with spraying of SL.4 instead of SL.1. Inventive granule Gr.4 was obtained.

### III.1: Comparative example: Manufacture of a comparative spray drying of copolymer (A)

A Sokalan® SR400 aqueous solution with a content of 31 % by weight was applied with a brush on a hot surface (150°C). After 10 minutes of drying time, the dried Sokalan® SR400 was still sticky and ruber-like. No powder or granules could be obtained even after prolonged drying.

### Storage tests:

A standard powder detergent was mixed with the inventive granules by a dry mixing equipment. The resulting products were stored and subjected to an olfactory assessment up to 12 weeks. The result is given as "pass" or "no pass".

| product | intial | 4 weeks RT | 8 weeks RT | 12 weeks RT |
|---|---|---|---|---|
| Standard powder detergent | pass | pass | pass | pass |
| Standard powder detergent plus + inventive granule 3 | pass | pass | pass | pass |
| Standard powder detergent plus + inventive granule 4 | pass | pass | pass | pass |

### Performance Tests:

Textile sheets made of cotton and polyester, previously equipped with altogether 60 standardised stains, were laundered in the laundry machine at 30 °C with wash fleets each containing 3.8 g/l of a laundry detergent W1, W2 and W3 of the composition as described in table1, and subsequently dried. The resulting brightness values (Y values) were determined. The laundry detergent containing an inventive combination of agents were superior to the laundry detergents without the inventive combination.

**Table 1: composition of laundry detergents (weight-%)**

| | W1 | W2 | W3 |
|---|---|---|---|
| inventive granule 1 | - | 0,25 | - |
| inventive granule 3 | - | - | 0,25 |
| Carboxymethylcellulose | 3 | 3 | 3 |
| HEDP-Na4 | 1 | 1 | 1 |
| Polyacrylate | 3 | 3 | 3 |
| Sodium silicate | 7 | 7 | 7 |
| Sodium carbonate | 21 | 21 | 21 |
| Defoamer | 0,1 | 0,1 | 0,1 |
| Sodium hydrogen carbonate | 10 | 10 | 10 |
| Sodium percarbonate | 12 | 12 | 12 |
| TAED | 4 | 4 | 4 |
| Enzyme | 0,8 | 0,8 | 0,8 |
| Perfume | 0,3 | 0,3 | 0,3 |
| Alkyl Benzene Sulfonic Acid, Na-salt | 13 | 13 | 13 |
| Fatty Alcohol Sulfate-Na | 3 | 3 | 3 |
| Soap | 0,1 | 0,1 | 0,1 |
| Optical brightener | 0,2 | 0,2 | 0,2 |
| Water, Sodium Sulfate, other Polymers | Ad 100 | Ad 100 | Ad 100 |

**Table 2: number of stains on which improved removal of stains was detected, compared to W1:**

| | Fat containing stains on polyester | Fat containing stains on cotton |
|---|---|---|
| W2 | 6 | 5 |
| W3 | 8 | 9 |

## Claims

1. Process for making a powder or granule containing
(A) at least one copolymer obtainable by polymerization of at least one monomer according to formula (I): in an amount of 1 to 70 mole%,
wherein n is ≥ 3
and
at least one monomer according to formula (II): in an amount of 30 to 99 mole%,
(B) at least one homo- or copolymer of (meth)acrylic acid, partially or fully neutralized with alkali,
wherein the weight ratio of (A) to (B) is from 20:80 to 80:20,
said process comprising the steps of
(a) mixing the at least one copolymer (A) and the at least one homo- or copolymer (B) in the presence of water,
(b) removing most of said water by spray-drying or spray granulation using a gas with an inlet temperature of at least 125°C.

2. Process according to claim 1, wherein said powder or granule contains in the range of from 40 - 75 % by weight copolymer (A) and 60 - 25 % by weight homo- or copolymer (B), percentages referring to the solids content of said powder or granule.

3. Process according to claim 1 or 2, wherein the copolymer (A) is selected from random copolymer obtainable by polymerization of at least one monomer according to formula (I): in an amount of 1 to 67 mole%,
wherein n is between 5 and 7 and
at least one monomer according to formula (II): in an amount of 30 to 99 mole%.

4. Process according to any of the preceding claims, wherein said homo- and copolymer (B) is selected from the per-sodium salts of polyacrylic acid.

5. Process according to any of the preceding claims, wherein said homo- or copolymer (B) has an average molecular weight M_{w} in the range of from 1,200 to 30,000 g/mol, determined by gel permeation chromatography and referring to the respective free acid.

6. Process according to any of the preceding claims wherein said homo- and copolymers (B) are selected from copolymers of (meth)acrylic acid and a comonomer bearing at least one sulfonic acid group per molecule.

7. Powder or granule containing
(A) at least one copolymer obtainable by polymerization of at least one monomer according to formula (I): in an amount of 1 to 70 mole%,
wherein n is ≥ 3
and
at least one monomer according to formula (II): in an amount of 30 to 99 mole%,
(B) at least one homo- or copolymer of (meth)acrylic acid, partially or fully neutralized with alkali,
wherein the weight ratio of (A) to (B) is from 20:80 to 80:20

8. Powder or granule according to claim 7, said powder or granule containing
(A) in the range of from 40 - 75 % by weight of at least one copolymer obtainable by polymerization of at least one monomer according to formula (I): in an amount of 1 to 70 mole%,
wherein n is ≥ 3
and
at least one monomer according to formula (II): in an amount of 30 to 99 mole%,
(B) in the range of from 60 - 25 % by weight of at least one homo- or copolymer of (meth)acrylic acid, partially or fully neutralized with alkali,
in molecularly disperse form, percentages referring to the solids content of said powder or granule.

9. Powder or granule according to claim 7 or 8 having a residual moisture content in the range of from 1 to 20 % by weight.

10. Powder or granule according to any of claims 7 to 9 having an average diameter in the range of from powders with an average particle diameter in the range of from 1 µm to less than 0.1 mm and from granules with an average particle diameter in the range of from 0.1 mm to 2 mm.

11. Powder or granule according to any of claims 7 to 10 wherein said homo- or copolymer (B) has an average molecular weight M_{w} in the range of from 1,200 to 30,000 g/mol, determined by gel permeation chromatography and referring to the respective free acid.

12. Powder or granule according to any of claims 7 to 11 wherein copolymer (A) is selected from a random copolymer obtainable by polymerization of at least one monomer according to formula (I): in an amount of 1 to 67 mole%,
wherein n is between 5 and 7
and
at least one monomer according to formula (II): in an amount of 30 to 99 mole%.

13. Powder or granule according to any of claims 7 to 12 wherein said homo- and copolymer (B) is selected from the per-sodium salts of polyacrylic acid.

14. Powder or granule according to any of claims 7 to 13 wherein said homo- and copolymers (B) are selected from copolymers of (meth)acrylic acid and a comonomer bearing at least one sulfonic acid group per molecule.

15. Cleaning agent, containing at least one powder or granule according to any of claims 7 to 14.

## Patentansprüche

1. Verfahren zur Herstellung eines Pulvers oder Granulats, das
(A) mindestens ein Copolymer, das durch Polymerisation von mindestens einem Monomer gemäß Formel (I): in einer Menge von 1 bis 70 Mol-%,
wobei n ≥ 3 ist,
und
mindestens einem Monomer gemäß Formel (II): in einer Menge von 30 bis 99 Mol-% erhältlich ist,
(B) mindestens ein Homo- oder Copolymer von (Meth)acrylsäure, das teilweise oder vollständig mit Alkali neutralisiert ist,
wobei das Gewichtsverhältnis von (A) zu (B) 20:80 bis 80:20 beträgt,
enthält, wobei das Verfahren folgende Schritte umfasst:
(a) Mischen des mindestens einen Copolymers (A) und des mindestens einen Homo- oder Copolymers (B) in Gegenwart von Wasser,
(b) Entfernen des größten Teils des Wassers durch Sprühtrocknen oder Sprühgranulieren unter Verwendung eines Gases mit einer Einlasstemperatur von mindestens 125 °C.

2. Verfahren nach Anspruch 1, wobei das Pulver oder Granulat im Bereich von 40-75 Gew.-% Copolymer (A) und 60-25 Gew.-% Homo- oder Copolymer (B) enthält, wobei sich die Prozentangaben auf den Feststoffgehalt des Pulvers oder Granulats beziehen.

3. Verfahren nach Anspruch 1 oder 2, wobei das Copolymer (A) aus statistischen Copolymeren, die durch Polymerisation von mindestens einem Monomer gemäß Formel (I): in einer Menge von 1 bis 67 Mol-%,
wobei n zwischen 5 und 7 liegt,
und
mindestens einem Monomer gemäß Formel (II): in einer Menge von 30 bis 99 Mol-% erhältlich ist, ausgewählt wird.

4. Verfahren nach einem der vorhergehenden Ansprüche, wobei das Homo- und Copolymer (B) aus den Pernatriumsalzen von Polyacrylsäure ausgewählt wird.

5. Verfahren nach einem der vorhergehenden Ansprüche, wobei das Homo- oder Copolymer (B) ein durch Gelpermeationschromatographie bestimmtes und sich auf die jeweilige freie Säure beziehendes mittleres Molekulargewicht M_{w} im Bereich von 1.200 bis 30.000 g/mol aufweist.

6. Verfahren nach einem der vorhergehenden Ansprüche, wobei die Homo- und Copolymere (B) aus Copolymeren von (Meth)acrylsäure und einem Comonomer mit mindestens einer Sulfonsäuregruppe pro Molekül ausgewählt werden.

7. Pulver oder Granulate, enthaltend
(A) mindestens ein Copolymer, das durch Polymerisation von mindestens einem Monomer gemäß Formel (I): in einer Menge von 1 bis 70 Mol-%,
wobei n ≥ 3 ist,
und
mindestens einem Monomer gemäß Formel (II): in einer Menge von 30 bis 99 Mol-% erhältlich ist,
(B) mindestens ein Homo- oder Copolymer von (Meth)acrylsäure, das teilweise oder vollständig mit Alkali neutralisiert ist,
wobei das Gewichtsverhältnis von (A) zu (B) 20:80 bis 80:20 beträgt.

8. Pulver oder Granulat nach Anspruch 7, wobei das Pulver oder Granulat
(A) im Bereich von 40-75 Gew.-% mindestens eines Copolymers, das durch Polymerisation von mindestens einem Monomer gemäß Formel (I): in einer Menge von 1 bis 70 Mol-%,
wobei n ≥ 3 ist,
und
mindestens einem Monomer gemäß Formel (II): in einer Menge von 30 bis 99 Mol-% erhältlich ist,
(B) im Bereich von 60-25 Gew.-% mindestens eines Homo- oder Copolymers von (Meth)acrylsäure, das teilweise oder vollständig mit Alkali neutralisiert ist,
in molekulardisperser Form enthält, wobei sich die Prozentangaben auf den Feststoffgehalt des Pulvers oder Granulats beziehen.

9. Pulver oder Granulate nach Anspruch 7 oder 8 mit einem Restfeuchtigkeitsgehalt im Bereich von 1 bis 20 Gew.-%.

10. Pulver oder Granulat nach einem der Ansprüche 7 bis 9 mit einem mittleren Durchmesser im Bereich von Pulvern mit einem mittleren Teilchendurchmesser im Bereich von 1 µm bis weniger als 0,1 mm und von Granulaten mit einem mittleren Teilchendurchmesser im Bereich von 0,1 mm bis 2 mm.

11. Pulver oder Granulate nach einem der Ansprüche 7 bis 10, wobei das Homo- oder Copolymer (B) ein durch Gelpermeationschromatographie bestimmtes und sich auf die jeweilige freie Säure beziehendes mittleres Molekulargewicht M_{w} im Bereich von 1.200 bis 30.000 g/mol aufweist.

12. Pulver oder Granulat nach einem der Ansprüche 7 bis 11, wobei das Copolymer (A) aus statistischen Copolymeren, die durch Polymerisation von mindestens einem Monomer gemäß Formel (I): in einer Menge von 1 bis 67 Mol-%,
wobei n zwischen 5 und 7 liegt,
und
mindestens einem Monomer gemäß Formel (II): in einer Menge von 30 bis 99 Mol-%
erhältlich ist, ausgewählt ist.

13. Pulver oder Granulat nach einem der Ansprüche 7 bis 12, wobei das Homo- und Copolymer (B) aus den Pernatriumsalzen von Polyacrylsäure ausgewählt ist.

14. Pulver oder Granulat nach einem der Ansprüche 7 bis 13, wobei die Homo- und Copolymere (B) aus Copolymeren von (Meth)acrylsäure und einem Comonomer mit mindestens einer Sulfonsäuregruppe pro Molekül ausgewählt sind.

15. Reinigungsmittel, enthaltend mindestens ein Pulver oder Granulat nach einem der Ansprüche 7 bis 14.

## Revendications

1. Procédé pour la préparation d'une poudre ou d'un granulé contenant
(A) au moins un copolymère qui peut être obtenu par polymérisation d'au moins un monomère selon la formule (I) : en une quantité de 1 à 70 % en moles,
n étant ≥ 3
et
d'au moins un monomère selon la formule (II) : en une quantité de 30 à 99 % en moles,
(B) au moins un homopolymère ou copolymère d'acide (méth)acrylique, partiellement ou totalement neutralisé avec un alcali,
le rapport en poids de (A) sur (B) étant de 20:80 à 80:20,
ledit procédé comprenant les étapes de
(a) mélange de l'au moins un copolymère (A) et de l'au moins un homopolymère ou copolymère (B) en la présence d'eau,
(b) élimination de la plupart de ladite eau par séchage par pulvérisation ou granulation par pulvérisation à l'aide d'un gaz doté d'une température d'entrée d'au moins 125 °C.

2. Procédé selon la revendication 1, ladite poudre ou ledit granulé contenant dans la plage allant de 40 à 75 % en poids de copolymère (A) et 60 à 25 % en poids d'homopolymère ou copolymère (B), les pourcentages faisant référence à la teneur en solides de ladite poudre ou dudit granulé.

3. Procédé selon la revendication 1 ou 2, le copolymère (A) étant choisi parmi un copolymère statistique qui peut être obtenu par polymérisation d'au moins un monomère selon la formule (I) : en une quantité de 1 à 67 % en moles,
n étant compris entre 5 et 7
et
d'au moins un monomère selon la formule (II) : en une quantité de 30 à 99 % en moles.

4. Procédé selon l'une quelconque des revendications précédentes, ledit homopolymère ou copolymère (B) étant choisi parmi les sels per-sodiques d'un poly(acide acrylique).

5. Procédé selon l'une quelconque des revendications précédentes, ledit homopolymère ou copolymère (B) possédant un poids moléculaire moyen M_{w} dans la plage allant de 1 200 à 30 000 g/mole, déterminé par chromatographie à perméation de gel et faisant référence à l'acide libre respectif.

6. Procédé selon l'une quelconque des revendications précédentes, lesdits homopolymères ou copolymères (B) étant choisis parmi des copolymères d'acide (méth)acrylique et d'un comonomère portant au moins un groupe de type acide sulfonique par molécule.

7. Poudre ou granulé contenant
(A) au moins un copolymère qui peut être obtenu par polymérisation d'au moins un monomère selon la formule (I) : en une quantité de 1 à 70 % en moles,
n étant ≥ 3
et
d'au moins un monomère selon la formule (II) : en une quantité de 30 à 99 % en moles, (B) au moins un homopolymère ou copolymère d'acide (méth)acrylique, partiellement ou totalement neutralisé avec un alcali,
le rapport en poids de (A) sur (B) étant de 20:80 à 80:20.

8. Poudre ou granulé selon la revendication 7, ladite poudre ou ledit granulé contenant
(A) dans la plage allant de 40 à 75 % en poids d'au moins un copolymère qui peut être obtenu par polymérisation d'au moins un monomère selon la formule (I) : en une quantité de 1 à 70 % en moles,
n étant ≥ 3
et
d'au moins un monomère selon la formule (II) : en une quantité de 30 à 99 % en moles,
(B) dans la plage allant de 60 à 25 % en poids d'au moins un homopolymère ou copolymère d'acide (méth)acrylique, partiellement ou totalement neutralisé avec un alcali,
sous forme dispersée sur le plan moléculaire, les pourcentages faisant référence à la teneur en solides de ladite poudre ou dudit granulé.

9. Poudre ou granulé selon la revendication 7 ou 8 possédant une teneur en humidité résiduelle dans la plage allant de 1 à 20 % en poids.

10. Poudre ou granulé selon l'une quelconque des revendications 7 à 9 possédant un diamètre moyen dans la plage allant de poudres dotées d'un diamètre moyen de particule dans la plage allant de 1 µm à moins de 0,1 mm et de granulés dotés d'un diamètre moyen de particule dans la plage allant de 0,1 mm à 2 mm.

11. Poudre ou granulé selon l'une quelconque des revendications 7 à 10, ledit homopolymère ou copolymère (B) possédant un poids moléculaire moyen M_{w} dans la plage allant de 1 200 à 30 000 g/mole, déterminé par chromatographie à perméation de gel et faisant référence à l'acide libre respectif.

12. Poudre ou granulé selon l'une quelconque des revendications 7 à 11, le copolymère (A) étant choisi parmi un copolymère statistique qui peut être obtenu par polymérisation d'au moins un monomère selon la formule (I) : en une quantité de 1 à 67 % en moles,
n étant compris entre 5 et 7
et
d'au moins un monomère selon la formule (II) : en une quantité de 30 à 99 % en moles.

13. Poudre ou granulé selon l'une quelconque des revendications 7 à 12, ledit homopolymère ou copolymère (B) étant choisi parmi des sels per-sodiques d'un poly(acide acrylique).

14. Poudre ou granulé selon l'une quelconque des revendications 7 à 13, lesdits homopolymères ou copolymères (B) étant choisis parmi des copolymères d'acide (méth)acrylique et d'un comonomère portant au moins un groupe de type acide sulfonique par molécule.

15. Agent de nettoyage, contenant au moins une poudre ou au moins un granulé selon l'une quelconque des revendications 7 à 14.
